

June 20, 1939.

R. H. GUINZBURG

WEARING APPAREL

Filed Jan. 14, 1936

2,162,810



INVENTOR  
ROLAND H. GUINZBURG.  
BY *Lawrence Leisner*  
ATTORNEY

Patented June 20, 1939

2,162,810

# UNITED STATES PATENT OFFICE

2,162,810

## WEARING APPAREL

Roland H. Guinzburg, Flushing, N. Y., assignor  
to I. B. Kleinert Rubber Company, New York,  
N. Y.

Application January 14, 1936, Serial No. 59,071

2 Claims. (Cl. 2—34)

The present invention relates to wearing apparel and, more particularly, to garments made of or including elastic material.

As heretofore constructed, such articles of 5 wearing apparel as baby pants, ladies' girdles, and other garments which are made wholly or partly of rubber, so as to be either waterproof or elastic or both waterproof and elastic, are subject to numerous objections. For example, ladies' girdles made of sheet rubber are open to the objection that the girdles have too much elasticity or extensibility in a longitudinal direction, that is, longitudinally of the wearer, because ordinary sheet rubber has substantially the same elasticity 10 or extensibility in all directions. On the other hand, the elasticity of a girdle in a direction longitudinally of the wearer should be limited and preferably substantially less than the elasticity of the girdle in a circumferential direction. Similarly, such garments as baby pants should preferably be elastic circumferentially of the wearer but of limited elasticity in a longitudinal direction.

Girdles possessing different elastic characteristics with respect to their circumferential and longitudinal directions have been produced by 25 making such girdles of elastic webbing, that is, of woven or knit textile material in which elastic strands are incorporated in such manner that 30 the girdle has the desired degree of elasticity circumferentially of the girdle and reduced elasticity longitudinally thereof. Such materials, besides being relatively expensive, are not entirely satisfactory and are unsuitable for certain purposes, particularly where the waterproof or air- 35 impervious quality of the material is desired, as for example, in such garments as baby pants and reducing girdles.

One object of the invention is the provision of 40 garments made of fluid-impervious sheet rubber material which is inherently elastically different in different directions.

Another object of the invention is the provision 45 of sheet rubber garments possessing different circumferential and longitudinal elasticities.

Another object of the invention is to provide a garment made of sheet rubber which is of high 50 flexibility and yet can be readily subjected to garment-manufacturing operations such as stitching or similar processes, thereby making it unnecessary to laminate rubber sheets with a textile fabric.

Another object of the invention is to provide 55 garments made of sheet rubber which, while of substantially reduced elasticity in one direction,

has substantially the same degree of flexibility as ordinary sheet rubber of the same thickness.

Another object of the invention is to provide a garment of sheet rubber material of such character as to provide a soft pleasant surface, thereby 5 eliminating the undesirable surface feel of ordinary sheet rubber.

The above objects of the invention and other objects ancillary thereto will best be understood from the following description considered in connection with the accompanying drawing.

In the drawing:

Fig. 1 is a front view of one type of garment, 10 namely, baby pants, made in accordance with the present invention;

Fig. 2 is a view of another type of garment, 15 namely, a lady's girdle, made in accordance with the present invention; and

Fig. 3 is a plan view of a piece of material, 20 showing a modification of the present invention.

The baby pants 10, shown in Fig. 1, and the lady's girdle 12, shown in Fig. 2, may be of any well known or preferred construction. In accordance with the present invention, however, both of these garments are made of thin sheet rubber 25 material which is substantially elastic in one direction and of reduced elasticity in another direction. More specifically, when a garment such as the baby pants 10 or the girdle 12 are made of the sheet rubber material of the present 30 invention, it has considerable elasticity or extensibility in a circumferential direction, that is, in a direction encircling the body of the wearer, but has substantially reduced elasticity in a longitudinal direction.

In accordance with the present invention, in 35 making said material, any suitable commercial rubber, as, for instance, "washed and dried" rubber, may be used. The rubber may be introduced into the processing either in the relatively unmanufactured condition in which it arrives from the plantation or other native source, or may have been advanced through the manufacturing 40 stages to become batched or broken down rubber. For instance, the rubber may have been 45 advanced, from the stage of the crepe type of plantation rubber, through one or more stages of a batching process, to prepare it for efficient processing in accordance with the invention. The batch is worked upon apparatus such as a mixing 50 mill, or a rubber masticator or like effect. The manner of this processing may follow substantially the usual course of manipulation used on mixing mills, especially in the first period where the rubber is broken up and softened for the sub- 55

sequent processing. While the rubber is feeding through the masticator or mill, and after an interval of about twenty minutes, depending upon the particular batch of rubber, customarily 5 voted to breaking down the rubber, there is introduced into the mass of rubber, for incorporation thereto, a quantity of flock. The proportions of flock may be varied in accordance with certain factors in the product desired, as, for 10 instance, the thickness of the sheet intended to be produced, and other factors of commercial importance.

The mixture thus produced is subjected to a sufficient mastication to effect, at this stage, substantially 15 complete incorporation of all the flock into, and uniform distribution of such flock throughout, the rubber. In this masticating operation, other compounds such as coloring matter may be introduced. It was found that, on the 20 mixing mill, fine grinding of the batched rubber and flock assisted in securing substantially uniform distribution, the end point of the mastication being reached by setting the rolls closely up toward each other, in one case so that they were 25 but about one-sixteenth inch apart.

The substance introduced at the mixing mill for the manufacture of this type of rubber may be described as extremely fine fibres, such, for instance, as are found in textile fibres. Such fine 30 fibres may be reduced to an even finer state than the normal condition in commerce, as, for instance, by grinding or by some similar operation. The particular fibres used in preparing certain 35 embodiments in accordance with the invention include fibres of the animal type, such as silk flock, and fibres of the cellulosic type, such as cotton flock, that is, fibres of silk and cotton which had been reduced to a very fine, powdery condition. In fact, this flock is as fine as flour, 40 so fine that the individual fibres are barely, if at all, visible to the naked eye. It has been found that the finer the flock used, the more accentuated are the results secured. Such fineness makes possible the production of very thin 45 sheets without pin holes. Also, the amount of flock introduced was found to be most effective when, into the masticator, there were introduced between eight to twenty parts of flock for each ninety-two to seventy-five parts of rubber and 50 other compounds. Rubber processed in this manner could be calendered into sheets between five one-thousandths and twenty-five one-thousandths of an inch, although only gauges between twelve one-thousandths and twenty one-thousandths were necessary for commercial use. 55 All of these factors can be arrived at without the introduction of any brittleness into the sheet.

After mastication, while the resultant rubber preferably is given the usual rest, it may immediately, or after such a rest, be removed to the calender rollers. While ordinary temperatures of calendering may suffice for the manufacture of a product within certain of the elements of this invention, it has been found that a slight rise in 60 the neighborhood of 10° F. to 20° F. resulted in an appreciable development of the desired properties of the product.

The mass of incorporated rubber and flock is calendered without any material change from 65 the method practiced by skilled calender crews who determine the condition of the rubber in the customary manner, considering the amount of flock and other introduced compounds. When the calendered mass finally has reached the desired 70 condition, the sheet is removed from the

rolls in the usual manner, and made up in readiness for vulcanization.

Even after the mixing operation, the rubber is found to have attained a degree of non-elasticity in the line in which it is removed from the rolls. This characteristic is found to be even more enhanced when the material passes, in its unvulcanized state, from the calender rolls.

Accordingly, the material when utilized for making such garments as baby pants and girdles, 10 is cut so that the direction of reduced elasticity is in the longitudinal direction of the garment or at right angles to the circumferential or body-encircling direction.

After calendering and preferably a suitable rest period, the sheet may be subjected to vulcanization. In this stage of processing, substantially any suitable method may be followed. However, the acid cure or vapor cure has been found most effective in delivering a rubber having the desired 15 characteristics. After vulcanization, the condition of unelasticity is found to be even more marked, and set in the sheet. However, flexibility is substantially unaffected, whereas toughness appears to be measurably increased. When 20 coloring matter is introduced, during processing, it takes effect uniformly and without difficulty. The sheet may be cut and formed into different articles of wearing apparel, and it may be 25 stitched, the stitches holding substantially as if 30 in a textile, and without tearing.

In making certain garments, such as the baby pants 10, the material may be cut and at least partly assembled in its unvulcanized state and subsequently vulcanized. Thus, in making the 35 garment 10, a sheet of the unvulcanized material may be cut to the desired pattern to provide the rear portion 14 and the front portion 16 provided with the leg openings 18. Also, the material may be cut to provide the openings 20 which improve 40 the fit of the garment. To form the garment 10, the side edges of the sheet are overlapped between the openings 18 and 20 at each side of the garment and secured together by subjecting them to the pressure of a knurling roller forming the 45 unstitched seams 22. If desired, a rubber cement may be used for forming said seams alternatively or additionally to the pressure of said roller. The garment is then vulcanized and subsequently, in order to shape the garment and to increase the 50 extensibility thereof at the waist and leg openings, the material may be gathered adjacent said openings and bindings 24 may be attached preferably by stitching of a well known character which permits the garment to expand and contract. Said bindings may be of any suitable material but are preferably formed from the material of the present invention cut from the sheet and arranged in the garment to be circumferentially elastic. The girdle 12 is formed preferably 55 from the vulcanized sheet material in accordance with any well known manufacturing method.

Sheet rubber material made in accordance with the above described process possesses considerable 60 elasticity in one direction although said material even in that one direction is somewhat less elastic than ordinary sheet rubber.

In accordance with a modification of the present invention, the sheet material is substantially 65 inelastic in both directions, thus making it possible to use such substantially inelastic fluid-impermeable material for making garments or parts thereof which are substantially inelastic. This is accomplished in accordance with the present in- 70 75

vention by combining two of the sheets in an unvulcanized state, after they are removed from the calender rolls. Referring to Fig. 3 of the drawing, the unvulcanized sheets A and B, each made as described above, are superposed on each other so that the direction of non-elasticity of the sheet A, as indicated by the double arrow on said sheet, is at right angles to the direction of non-elasticity of the sheet B, as indicated by the double arrow on the last mentioned sheet. Then the superposed sheets are passed through calender rolls which cause them to be firmly united with each other throughout their contacting surfaces so that it is practically impossible to distinguish one pre-formed sheet from the other, the two sheets being welded together and forming, in effect, a sheet of single thickness. Finally, the sheet material thus produced is vulcanized, and the resulting product is substantially inelastic in both directions. It is within the scope of the present invention to make any of the garments of the class described, including the garments 10 and 12, wholly or partially of this material.

While I have shown and described several of the preferred embodiments of the invention, it will be understood that the invention is capable of being embodied otherwise than as herein shown and described and that certain changes in the particular composition of the material and in the steps of the process of making the latter may be made without substantially departing from the invention. Accordingly, the present description and drawing are to be considered as illus-

trative of the invention, and I do not wish to be limited thereto except as may be required by the appended claims considered with reference to the prior art.

Having thus described my invention, what I desire to claim and secure by Letters Patent of the United States is:

1. A reducing girdle comprising a member adapted to encircle the body of the wearer and composed of thin, flexible and elastic sheet material comprising sheet rubber having finely divided flock incorporated therein and being substantially more elastic in one direction than in another at right angles to said first direction, said material being arranged in the girdle so that said body encircling member is substantially elastic circumferentially thereof and is substantially less elastic in a longitudinal direction.

2. A garment of the class described comprising a member adapted to encircle the body of the wearer and which possesses substantial elasticity circumferentially and limited elasticity longitudinally, said member being made of thin sheet rubber material having finely divided textile flock incorporated therein and being inherently uniformly elastic in one direction and inherently of uniformly reduced elasticity in another direction, said material being cut and arranged in the garment so that said body encircling member is substantially elastic circumferentially thereof and substantially less elastic in a longitudinal direction.

ROLAND H. GUINZBURG.